

L. E. RIVOT.

Treating Ores.

No. 42,997.

Patented May 31, 1864.



Processes.

John  
J. L. Combe

Inventor

L. Rivot  
or  
M. L. Rivot

# UNITED STATES PATENT OFFICE.

LOUIS EDOUARD RIVOT, OF PARIS, FRANCE, ASSIGNOR TO JACQUES GAIL-LARDON, OF SAN FRANCISCO, CALIFORNIA.

## IMPROVEMENT IN TREATING AURIFEROUS AND ARGENTIFEROUS ORES.

Specification forming part of Letters Patent No. 42,997, dated May 31, 1864.

*To all whom it may concern:*

Be it known that I, LOUIS EDOUARD RIVOT, professor at the Imperial School of Mines in Paris, in the Empire of France, have invented a new and useful Process of Heating Auriferous and Argentiferous Ores; and I hereby declare the following, taken in connection with the accompanying drawings, is a full, clear, and exact description of the same.

My invention relates more particularly to the treatment of such ores containing metallic sulphurates and also selenides, tellurides, and other composites containing arsenic and antimony, which, when treated according to the various methods of amalgamation heretofore in use, fail to give favorable or practically good results; and my invention consists in a new method of treating such ores comprising the following operations: first, the grinding and porphyritization of ores mixed intimately with pyrites of iron or copper; second, the roasting of the ores by means of superheated steam; third, the amalgamation of the roasted ores; fourth, the separation of the amalgam; fifth, the compression of the amalgam; sixth, the distillation of the mercury; seventh, the fusion of the precious metal ores.

I shall now refer to each operation separately, and describe the manner in which the same is or may be carried into effect.

First. The grinding and porphyritization of the ores mixed with pyrites of iron or copper in proportions varying according to the composition of the ores. Any of the known machines or apparatus for grinding or triturating ores or other hard substances may be used for this operation.

Second. The roasting of the porphyritized ores mixed with pyrites by submitting the same to the action of steam superheated to a temperature somewhat above dark red, effected in an oven or furnace, of an arrangement new in metallurgy and represented in the accompanying drawing, in which—

Third. Figure 1 is a longitudinal elevation of the furnace; Fig. 2, a section on line 1 2; Fig. 3, another section on line 3, 4, 5, and 6; Fig. 4, a transverse section on line 7 8, and Fig. 5 is an end view on the side of the fire-chamber.

Above the sole A, and in the vicinity of the fire-chamber, there are arranged in the masonry

horizontal tuyeres *t*, containing blast-pipes *b*, whose orifices are rectangular, for the purpose of facilitating the expansion of the steam in sheet form upon the ore. The steam used should be introduced at a pressure at least one atmosphere over and above that of the surrounding medium. The pipes *T*, which supply the steam to the blast-pipes *b*, are provided with cocks *c* to regulate the quantity of the steam, and are branched upon a main pipe, *S*. Underneath the sole there is an arched reservoir, *B*, into which the roasted ores drop by passing through openings that are kept closed during the operation by means of cast-iron doors or plates. Immediately in rear of the furnace proper there is arranged the great condensing chamber *c*, wherein the arsenical and antimonial vapors or fumes are collected. The arrangement shown for the grate and fire-chamber is most suited for wood. Other fuel capable of producing a long flame may be used by applying slight modifications, which will readily suggest themselves. The length and width of the sole are varied according to the charge of ore for each operation.

The furnace of which the above is a description presents the following peculiarity and novelty: The ore being charged in thin layers upon the sole, the heating is effected by the reverberation of the roof, whose arch is followed by the flame in its course from the fire-bridge to the neck, while the roasting proper is produced by a jet of steam heated to dark red outside of and before being admitted into the reverberatory furnace. The steam is then entered the furnace through five or six tuyeres, *t*, disposed on either side of the fire-bridge. It is generated and heated to the required temperature in any known or convenient apparatus.

The object of the roasting by means of steam is to expel the arsenic, antimony, tellurides, selenides, and the sulphur from the ore in a state of volatilizable combination and to leave upon the hearth or sole of the furnace the silver or gold in a metallic state, and the other metals as oxides, together with the earthy gangues. The furnace is charged at the side through openings *E E'*, or the ore may be introduced through a hopper arranged in the middle of the roof. Either plan may

be adopted as most convenient. The *modus operandi* is very simple. The supply of steam is regulated in such manner as that it shall form a continuous sheet interposed between the flame and the ore. From time to time it is necessary to work the ore, so as to successively expose all the particles to contact with and action of the steam. When the roasting is completed, the ore is dropped down under the arched roof through the orifices *h*. The work is or may be continuous—that is to say, a new charge may be introduced as soon as the preceding charge is allowed to drop into the reservoir underneath the hearth.

The amalgamation of the roasted ore is effected in the manner as follows: The ore is put together with water and without addition of salt or of the magistral in large wooden barrels, revolving upon horizontal axles. These barrels should be arranged so that each can be rotated or stopped at will independently of the others. To the ore and water they contain are then added mercury and hard round stones. The object of this is to divide the mercury and to put it in prolonged and intimate contact with all the particles of the roasted ore, so that it may form amalgams with the silver and gold therein contained. When this is accomplished the barrels are rotated with less speed, and a fresh quantity of mercury is added for the purpose of uniting the amalgam in liquid globules, according to the excess of mercury.

*Fourth, separation of the amalgam:* The barrels last referred to are emptied of their contents—*i. e.*, of the liquid amalgam, the metallic oxides, and the earthy gangues. The sediments, which are composed of the oxides and the gangues, are carefully washed to extract from them the minute globules of amalgam and mercury that are usually by them retained. If the ore contains copper, or if, for the purpose of wasting by means of steam above referred to, pyrites of copper have been used, then the sediments or mud should be preserved, as they constitute a valuable copper ore.

*Fifth, compression of the amalgam:* The liquid amalgam is compressed in bags, or if a hydraulic press be used a pressure might be produced sufficient to squeeze the mercury not combined with either gold or silver out through the pores of close-textured cloth or wood.

*Sixth, distillation of mercury:* The result of the preceding operation, which is an amalgam nearly solid, is submitted to distillation, where by the mercury is volatilized in apparatus, collecting and condensing its vapors.

*Seventh, fusion of the precious metal:* The metal obtained by the preceding operation may be melted into ingots, and the silver and gold may be separated at the same time.

Ores containing bromide, chloride, or iodide of silver may be treated according to the process above described, either alone or in com-

bination with black sulphurous ores or with pyrites of iron or copper. There is no loss whatsoever from volatilization, and the whole of the metal is reduced to a metallic state.

The last three operations may be effected by any process of amalgamation known and in apparatus familiar to metallurgists.

From the above description of my invention it will be seen that the divers operations are either borrowed from processes well known or are devised in imitation of methods much less known. Thus the grinding and porphyritization of the ores, the separation of the amalgam from the residuary mud oxidated, the compression of the amalgam, the distillation of the mercury, the fusion of the precious metals are effected according to processes and by means of apparatus which are well known, and consequently belong to the public. On the other hand, the roasting by means of steam superheated in a reverberatory furnace of ores mixed with pyrites without the aid or intervention of reagents, such as salts and the magistral, are operations heretofore unknown or untried in metallurgical industry, although they are known in the science. Mentioning only what has been done in France, M. Regnault has studied many years ago the action of steam or metallic sulphurets, but his experiments have never been put in practice. More recently M. Cumenge (Ingénieur des Mines) has published in the *Annales des Mines* the result of his laboratory experiments on the steam action.

M. Cumenge has made an important step in demonstrating the necessity of mixing the argentiferous and auriferous ores with pyrites. There was still an important and useful step to make, the steam being used practically by this new method, which consists in the use of superheated steam, and a new and convenient disposition of the reverberatory furnace. The superheating of steam renders its action more powerful and rapid, and does away with the objection heretofore urged against its employment, which was that of its sluggishness or slowness of action. Again, the amalgamation by trituration of the ore with mercury and without reagents has never been attempted in metallurgical operations, because of the silver and gold in ores could not be made directly to combine with mercury. This direct amalgamation is rendered possible only by the combining with it of the process of roasting described, the main object being the reduction of the gold and silver to a metallic state, allowing the other metals to pass off as oxides upon which mercury has no action.

Having thus fully described my said invention and the manner in which the same is or may be carried into effect, I claim—

1. The roasting by means of superheated steam of auriferous and argentiferous ores, when combined or mixed with pyrites of iron or copper, substantially as set forth.

2. The general arrangement and construction of reverberatory furnaces adapted for

the roasting of ores by means of steam superheated, as hereinbefore described.

3. The process of amalgamation without reagents, substantially as hereinbefore described, whereby the roasting of ores may be rendered practicable and economical, as set forth.

In testimony whereof I have signed my name to this specification before two subscribing witnesses.

L. E. RIVOT.

Witnesses:

E. RICHARDS.

E. HERMAN GOULDS.